



US008778582B2

(12) **United States Patent**  
**Sweeney et al.**

(10) **Patent No.:** **US 8,778,582 B2**  
(b5) **Date of Patent:** **Jul. 15, 2014**

(54) **TONER COMPOSITIONS**(71) Applicant: **Xerox Corporation**, Norwalk, CT (US)(72) Inventors: **Maura A. Sweeney**, Irondequoit, NY (US); **Robert D. Bayley**, Fairport, NY (US); **Grazyna E. Kmiecik-Lawrynowicz**, Fairport, NY (US); **Brian S. Wang**, Webster, NY (US)(73) Assignee: **Xerox Corporation**, Norwalk, CT (US)

(\* ) Notice: Subject to any disclaimer, the term of this patent is extended or adjusted under 35 U.S.C. 154(b) by 15 days.

(21) Appl. No.: **13/666,856**(22) Filed: **Nov. 1, 2012**(65) **Prior Publication Data**

US 2014/0120467 A1 May 1, 2014

(51) **Int. Cl.****G03G 9/08** (2006.01)  
**G03G 9/097** (2006.01)(52) **U.S. Cl.**CPC ..... **G03G 9/09708** (2013.01); **G03G 9/0804** (2013.01); **G03G 9/0825** (2013.01)USPC ..... **430/108.1**; 430/108.2; 430/137.14(58) **Field of Classification Search**CPC G03G 9/09708; G03G 9/0804; G03G 9/0825  
USPC ..... 430/108.1, 108.2, 137.14  
See application file for complete search history.(56) **References Cited**

## U.S. PATENT DOCUMENTS

2,874,063 A 2/1959 Greig  
3,590,000 A 6/1971 Palermi et al.

|               |         |                              |
|---------------|---------|------------------------------|
| 3,655,374 A   | 4/1972  | Palermi et al.               |
| 3,720,617 A   | 3/1973  | Chatterji et al.             |
| 3,983,045 A   | 9/1976  | Jugle et al.                 |
| 4,265,990 A   | 5/1981  | Stolka et al.                |
| 4,563,408 A   | 1/1986  | Lin et al.                   |
| 4,584,253 A   | 4/1986  | Lin et al.                   |
| 4,935,326 A   | 6/1990  | Creatura et al.              |
| 4,937,166 A   | 6/1990  | Creatura et al.              |
| 5,223,368 A   | 6/1993  | Ciccarelli et al.            |
| 5,227,460 A   | 7/1993  | Mahabadi et al.              |
| 5,324,613 A   | 6/1994  | Ciccarelli et al.            |
| 5,346,797 A   | 9/1994  | Kmiecik-Lawrynowicz et al.   |
| 5,364,729 A   | 11/1994 | Kmiecik-Lawrynowicz et al.   |
| 5,403,693 A   | 4/1995  | Patel et al.                 |
| 5,418,108 A   | 5/1995  | Kmiecik-Lawrynowicz et al.   |
| 5,501,935 A   | 3/1996  | Patel et al.                 |
| 5,527,658 A   | 6/1996  | Hopper et al.                |
| 5,585,215 A   | 12/1996 | Ong et al.                   |
| 5,650,255 A   | 7/1997  | Ng et al.                    |
| 5,650,256 A   | 7/1997  | Veregin et al.               |
| 5,916,725 A * | 6/1999  | Patel et al. .... 430/137.14 |
| 6,004,714 A   | 12/1999 | Ciccarelli et al.            |
| 6,165,668 A   | 12/2000 | Wilson et al.                |

(Continued)

## FOREIGN PATENT DOCUMENTS

|    |         |         |
|----|---------|---------|
| EP | 1383011 | 7/2002  |
| EP | 1426830 | 12/2002 |

Primary Examiner — Mark A Chapman

(74) Attorney, Agent, or Firm — Pillsbury Winthrop Shaw Pittman LLP

(57) **ABSTRACT**

A toner having charge control agents which impart excellent triboelectric charging characteristics. In embodiments, the toner particles are made by a process in which the toner particles are made without a shell which provides homogeneous distribution of the charge control agents, providing a toner with higher charge and better environmental stability.

**17 Claims, 1 Drawing Sheet**

(56)

**References Cited**

U.S. PATENT DOCUMENTS

6,190,815 B1 2/2001 Ciccarelli et al.  
6,221,550 B1 4/2001 Wilson et al.  
6,652,634 B1 11/2003 Akers, Jr. et al.

2004/0002014 A1 1/2004 Chae et al.  
2008/0261137 A1 \* 10/2008 Qin et al. .... 430/108.3  
2009/0047593 A1 2/2009 Vanbesien et al.  
2011/0117486 A1 \* 5/2011 Bayley et al. .... 430/108.24

\* cited by examiner



**1**  
**TONER COMPOSITIONS**

**BACKGROUND**

The present disclosure relates to toners and processes useful in providing toners suitable for electrophotographic apparatuses, including apparatuses such as digital, image-on-image, and similar apparatuses. In particular, the present embodiments are directed to a process for making toners that increases the charge of the toner particles, and toners made from the same.

Numerous processes are within the purview of those skilled in the art for the preparation of toners. Emulsion aggregation (EA) is one such method. These toners are within the purview of those skilled in the art and toners may be formed by aggregating a colorant with a latex polymer formed by emulsion polymerization. For example, U.S. Pat. No. 5,853,943, the disclosure of which is hereby incorporated by reference in its entirety, is directed to a semi-continuous emulsion polymerization process for preparing a latex by first forming a seed polymer. Other examples of emulsion/aggregation/coalescing processes for the preparation of toners are illustrated in U.S. Pat. Nos. 5,403,693, 5,418,108, 5,364,729, and 5,346,797, the disclosures of each of which are hereby incorporated by reference in their entirety. Other processes are disclosed in U.S. Pat. Nos. 5,527,658, 5,585,215, 5,650, 255, 5,650,256 and 5,501,935, the disclosures of each of which are hereby incorporated by reference in their entirety.

Toner systems normally fall into two classes: two component systems, in which the developer material includes magnetic carrier granules having toner particles adhering triboelectrically thereto; and single component systems (SDC), which may use only toner. Placing charge on the particles, to enable movement and development of images via electric fields, is most often accomplished with triboelectricity. Triboelectric charging may occur either by mixing the toner with larger carrier beads in a two component development system or by rubbing the toner between a blade and donor roll in a single component system.

Charge control agents (CCA) may be utilized to enhance triboelectric charging. Charge control agents may include organic salts or complexes of large organic molecules. Such agents may be applied to toner particle surfaces by a blending process. Such charge control agents may be used in small amounts of from about 0.01 weight percent to about 5 weight percent of the toner to control both the polarity of charge on a toner and the distribution of charge on a toner. Although the amount of charge control agents may be small compared to other components of a toner, charge control agents may be important for triboelectric charging properties of a toner. These triboelectric charging properties, in turn, may impact imaging speed and quality, as well as allow for extended life performance. Examples of charge control agents include those found in EP Patent Application No. 1426830, U.S. Pat. No. 6,652,634, EP Patent Application No. 1383011, U.S. Patent Application Publication No. 2004/0002014, U.S. Patent Application Publication No. 2003/0191263, U.S. Pat. No. 6,221,550, and U.S. Pat. No. 6,165,668, the disclosures of each of which are totally incorporated herein by reference.

One issue that may arise with charge control agents is that they are difficult to incorporate into emulsion aggregation toners. Generally, during incorporation some charging properties are lost. Namely, the charging property is no longer evident when the additive package is added to the particle, causing a drastic decrease in charge and thus ultimately impacting life performance of the toner.

**2**

Moreover, current toner formulations show that charging is zone specific, performing with stability in B zone and J Zone but worsening in A Zone. Through the addition of a shell to the toner particle, passivation of the pigments is possible but if a charge control agent is added to the core, shell or both, the charge control agent tends to create inhomogeneity of the charging. This is due to the fact that the addition of charge control agents in the shell tends to cause non-homogenous distribution of the charge control agent, and thus, leads to inhomogeneity of the charging. Compounding the problem is the fact that high amounts of residual surfactant also contribute to zone variability in the charging. Because most emulsion aggregate toner is made with nano-sized pigment, wax and latex, all of these substituents must be dispersed using high surfactant levels. An issue with this method is that too much surfactant causes issues with zone charging from J zone to A zone to B zone.

Thus, improved methods for producing toner, which permit excellent control of the charging of toner particles, remain desirable.

**SUMMARY**

According to aspects illustrated herein, there is provided a toner comprising shell-less toner particles comprising a core portion comprising a resin, wax and colorant, and a charge control agent distributed homogeneously throughout the core portion.

In another embodiment, there is provided a process for a toner comprising shell-less toner particles comprising a core portion comprising a resin, wax and colorant, a charge control agent distributed homogeneously throughout the core portion, and a residual surfactant on a surface of the core portion.

In yet further embodiments, there is provided a process for producing toner comprising: adding and mixing a colorant, a wax, and a charge control agent to an emulsion comprising at least one resin to form toner particles; aggregating the particles to form aggregated particles; and coalescing the aggregated particles to form shell-less toner particles comprising a core portion comprising a resin, wax and colorant, and a charge control agent distributed homogeneously throughout the core portion.

**BRIEF DESCRIPTION OF THE DRAWINGS**

FIG. 1 is a schematic diagram illustrating the process of producing a shell-less toner according to the present embodiments.

**DETAILED DESCRIPTION OF EMBODIMENTS**

The present disclosure provides toners and processes for the preparation of toner particles having excellent charging characteristics. It has been discovered that, by making an emulsion aggregate toner without the shell, more charge control agent is present in the toner and at the surface for charging stability throughout all zones. Furthermore, by adjusting the emulsion aggregation process and increasing the amount of charge control agent incorporated into the core-type particle (without the shell), more charge control agent is exposed and available and less surfactant is present to impact the higher humidity zones. As a result, the present embodiments provide an improved process for incorporating polymerized internal charge control agents and reducing the surfactant level in toners, especially emulsion aggregate toners, to provide higher charge and improved environmental charging stability.

The present embodiments thus provide a toner formulation and a process for producing the same in which a charge control agent is incorporated into a toner particle without a shell. By eliminating the shell formation step, and then washing, the charge control agent is better incorporated into the particle core and the surfactants are more readily removed. It is believed that the shell may encapsulate the surfactants and prevent their removal during washing.

In embodiments, toners of the present disclosure may be prepared by combining a latex polymer with an optional colorant, an optional wax, and other optional additives. In embodiments, the CCA is added to a latex, colorant, wax, and other additives to incorporate the CCA within the toner particles. While the latex polymer may be prepared by any method within the purview of those skilled in the art, in embodiments the latex polymer may be prepared by emulsion polymerization methods, including semi-continuous emulsion polymerization, and the toner may include emulsion aggregation toners. Emulsion aggregation involves aggregation of submicron latex, wax and pigment particles into toner size particles, where the growth in average particle size is, for example, in embodiments from about 0.1 micron to about 15 microns, or from about 1.5 to about 10 microns, or from about 3.5 to about 8 microns.

As shown in FIG. 1, the process of the present embodiments comprises combining and initial mixing of a charge control agent, polymeric resin, wax and pigment 5, followed by the aggregation of these components 10, and then coalescence 15 to achieve the proper toner shape without the shell to hinder charging of the charge control latex.

While the toner may be of any type, in specific embodiments, the toner is an emulsion aggregation toner. It was demonstrated that formulation of the toner particle was optimized using the emulsion/aggregation process. The toner may have a particle shape including, circular, needle-like, potato, raspberry and mixtures thereof. In embodiments, the toner particles may have a circularity of from about 0.940 to about 0.999, or from about 0.950 to about 0.995, or from about 0.960 to about 0.990.

#### Charge Control Agents

Suitable charge control agents which may be utilized include, in embodiments, metal complexes of alkyl derivatives of acids such as salicylic acid, other acids such as dicarboxylic acid derivatives, benzoic acid, oxynaphthoic acid, sulfonic acids, other complexes such as polyhydroxyalcanoate quaternary phosphonium trihalozincate, metal complexes of dimethyl sulfoxide, combinations thereof, and the like. Metals utilized in forming such complexes include, but are not limited to, zinc, manganese, iron, calcium, zirconium, aluminum, chromium, combinations thereof, and the like. Alkyl groups which may be utilized in forming derivatives of salicylic acid include, but are not limited to, methyl, butyl, t-butyl, propyl, hexyl, combinations thereof and the like. Examples of such charge control agents include those commercially available as BONTRON® E-84 and BONTRON® E-88 (commercially available from Orient Chemical). BONTRON® E-84 is a zinc complex of 3,5-di-tert-butylsalicylic acid in powder form. BONTRON® E-88 is a mixture of hydroxyaluminium-bis[2-hydroxy-3,5-di-tert-butylbenzoate] and 3,5-di-tert-butylsalicylic acid. Other suitable CCAs include the calcium complex of 3,5-di-tert-butylsalicylic acid, a zirconium complex of 3,5-di-tert-butylsalicylic acid, and an aluminum complex of 3,5-di-tert-butylsalicylic acid, as disclosed in U.S. Pat. Nos. 5,223,368 and 5,324,613, the disclosures of each of which are incorporated by reference in their entirety, combinations thereof, and the like.

In specific embodiments, the charge control agent is a zinc or aluminum-type salicyclic acid polymeric charge control agent, such as for example, zinc and aluminum 3,5-ditertiary butyl salicylic acid. In embodiments, the charge control agent is present in an amount of from about 0.05 to about 10 percent, or of from about 0.1 to about 5 percent, or of from about 0.15 to about 3 percent by weight of the total weight of the toner particle. In embodiments, the resulting toner has increased bulk and surface levels of the charge control agent and lower levels of surfactant. The toner also exhibits higher charge level in A zone. For example, the toner may have a triboelectric charge of from about -10 to about 80 uC/gm or from about -15 to about -60 uC/gm or from about -20 to about -40 uC/gm in A zone.

Specifically, the bulk level of the charge control agent is from about 0.05 to about 15 percent, or of from about 0.1 to about 10 percent, or of from about 0.2 to about 5 percent by weight of the total weight of the toner particle. As used herein, the "bulk level" is defined as the level of CCA throughout the particle, both core and shell. Such amounts are an increase of from about 0.1 to about 20 percent, or of from about 0.25 to about 15 percent, or of from about 0.75 to about 10 percent as compared to the bulk level of a toner particle prepared with the shell. The surface level of the charge control agent is from about 0.001 to about 10 percent, or of from about 0.01 to about 5 percent, or of from about 0.1 to about 2.5 percent by weight of the total weight of the toner particle. As used herein, the "surface level" is defined as the level of CCA measured on the toner particle surface and not in the bulk toner. Such amounts are an increase of from about 0.01 to about 10 percent, or of from about 0.1 to about 5 percent, or of from about 0.5 to about 2.5 percent as compared to the surface level of a toner particle prepared with the shell.

In the present embodiments, the charge control agent is spread or distributed homogeneously throughout the toner particle, including the core portion. As used herein, "homogeneous" means uniform composition throughout. Thus, in the present embodiments, the charge control agent is distributed uniformly throughout the toner particles, including the core portion. In embodiments, the homogeneity of the charge control distribution is from about 1 to about 98 percent, or from about 5 to about 78 percent, or from about 10 to about 68 percent, with 100% indicating complete homogeneity. The present embodiments achieve from about 0.1 to about 99 percent, or from about 10 to about 94 percent, or from about 20 to about 90 percent greater homogeneity than a toner particle prepared with the shell.

#### Resin

Any monomer suitable for preparing a latex for use in a toner may be utilized. As noted above, in embodiments the toner may be produced by emulsion aggregation. Suitable monomers useful in forming a latex polymer emulsion, and thus the resulting latex particles in the latex emulsion, include, but are not limited to, styrenes, acrylates, methacrylates, butadienes, isoprenes, acrylic acids, methacrylic acids, acrylonitriles, combinations thereof, and the like.

In embodiments, the latex polymer may include at least one polymer. In embodiments, at least one may be from about one to about twenty and, in embodiments, from about three to about ten. Exemplary polymers include styrene acrylates, styrene butadienes, styrene methacrylates, and more specifically, poly(styrene-alkyl acrylate), poly(styrene-1,3-diene), poly(styrene-alkyl methacrylate), poly(styrene-alkyl acrylate-acrylic acid), poly(styrene-1,3-diene-acrylic acid), poly(styrene-alkyl methacrylate-acrylic acid), poly(alkyl methacrylate-alkyl acrylate), poly(alkyl methacrylate-aryl acrylate), poly(aryl methacrylate-alkyl acrylate), poly(alkyl

methacrylate-acrylic acid), poly(styrene-alkyl acrylate-acrylonitrile-acrylic acid), poly(styrene-1,3-diene-acrylonitrile-acrylic acid), poly(alkyl acrylate-acrylonitrile-acrylic acid), poly(styrene-butadiene), poly(methylstyrene-butadiene), poly(methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), poly(butyl acrylate-isoprene), poly(styrene-propyl acrylate), poly(styrene-butyl acrylate), poly(styrene-butadiene-acrylic acid), poly(styrene-butadiene-methacrylic acid), poly(styrene-butadiene-acrylonitrile-acrylic acid), poly(styrene-butyl acrylate-acrylic acid), poly(styrene-butyl acrylate-methacrylic acid), poly(styrene-butyl acrylate-acrylonitrile), poly(styrene-butyl acrylate-acrylonitrile-acrylic acid), poly(styrene-butadiene), poly(styrene-isoprene), poly(styrene-butyl methacrylate), poly(styrene-butyl acrylate-acrylic acid), poly(butyl methacrylate-butyl acrylate), poly(butyl methacrylate-acrylic acid), poly(acrylonitrile-butyl acrylate-acrylic acid), and combinations thereof. The polymers may be block, random, or alternating copolymers.

In addition, polyester resins may be used as the latex polymer. Suitable polyesters which may be used include those obtained from the reaction products of bisphenol A and propylene oxide or propylene carbonate, as well as the polyesters obtained by reacting those reaction products with fumaric acid (as disclosed in U.S. Pat. No. 5,227,460, the entire disclosure of which is incorporated herein by reference), and branched polyester resins resulting from the reaction of dimethylterephthalate with 1,3-butanediol, 1,2-propanediol, and pentaerythritol. In embodiments, combinations of polyester resins, including amorphous polyester resins and crystalline polyester resins, may be utilized. Examples of such polyesters include those disclosed in U.S. Patent Application Publication No. 2009/0047593, the disclosure of which is hereby incorporated by reference in its entirety.

In embodiments, a poly(styrene-butyl acrylate) may be utilized as the latex polymer. The glass transition temperature of this latex, which in embodiments may be used to form a toner of the present disclosure, may be from about 35° C. to about 75° C., in embodiments from about 40° C. to about 70° C., in embodiments from about 45° C. to about 65° C.

In embodiments, the resin used to form a toner may have a weight average molecular weight (Mw) of from about 25 kpse to about 75 kpse, in embodiments from about 30 kpse to about 55 kpse, in other embodiments from about 35 kpse to about 55 kpse. The resin used to form a toner may have a number average molecular weight (Mn) of from about 1 kpse to about 30 kpse, in embodiments from about 2 kpse to about 20 kpse, in other embodiments from about 3 kpse to about 15 kpse. The polydispersity of the resin, i.e., Mw/Mn, may thus be of from about 0.5 to about 15, in embodiments from about 0.75 to about 10, in other embodiments from about 1 to about 5. The amount resin present in the toner may thus be of from about 50% wt/wt to about 90% wt/wt, in further embodiments from about 65% wt/wt to about 85% wt/wt, in other embodiments from about 70% wt/wt to about 80% wt/wt.

#### Surfactants

In embodiments, the latex may be prepared in an aqueous phase containing a surfactant or co-surfactant. Surfactants

which may be utilized with the polymer to form a latex dispersion can be ionic or nonionic surfactants, or combinations thereof, in an amount of from about 0.01 to about 15 weight percent of the solids, in embodiments of from about 0.1 to about 10 weight percent of the solids, in embodiments from about 1 to about 7.5 weight percent solids.

Anionic surfactants which may be utilized include sulfates and sulfonates, sodium dodecylsulfate (SDS), sodium dodecylbenzene sulfonate, sodium dodecylnaphthalene sulfate, dialkyl benzenealkyl sulfates and sulfonates, acids such as abietic acid available from Aldrich, NEOGEN R™, NEOGEN SCT™ obtained from Daiichi Kogyo Seiyaku Co., Ltd., combinations thereof, and the like.

Examples of cationic surfactants include, but are not limited to, ammoniums, for example, alkylbenzyl dimethyl ammonium chloride, dialkyl benzenealkyl ammonium chloride, lauryl trimethyl ammonium chloride, alkylbenzyl methyl ammonium chloride, alkyl benzyl dimethyl ammonium bromide, benzalkonium chloride, C12, C15, C17 trimethyl ammonium bromides, combinations thereof, and the like. Other cationic surfactants include cetyl pyridinium bromide, halide salts of quaternized polyoxyethylalkylamines, dodecylbenzyl triethyl ammonium chloride, MIRAPOL and ALKAQUAT available from Alkaril Chemical Company, SANISOL (benzalkonium chloride), available from Kao Chemicals, combinations thereof, and the like. In embodiments a suitable cationic surfactant includes SANISOL B-50 available from Kao Corp., which is primarily a benzyl dimethyl alkonium chloride.

Examples of nonionic surfactants include, but are not limited to, alcohols, acids and ethers, for example, polyvinyl alcohol, polyacrylic acid, methalose, methyl cellulose, ethyl cellulose, propyl cellulose, hydroxylethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, dialkylphenoxy poly(ethyleneoxy) ethanol, combinations thereof, and the like. In embodiments commercially available surfactants from Rhone-Poulenc such as IGEPAL CA-210™, IGEPAL CA-520™, IGEPAL CA-720™, IGEPAL CO-890™, IGEPAL CO-720™, IGEPAL CO-290™, IGEPAL CA-210™, ANTAROX 890™ and ANTAROX 897™ can be utilized.

In embodiments, the amount of surfactant present in the toner particle is reduced. Specifically, the amount of surfactant present in the toner particle is from about 1 to about 70 percent, or of from about 3 to about 60 percent, or of from about 5 to about 50 percent by weight of the total weight of the toner particle. Such amounts are a decrease of from about 30 to about 98 percent, or of from about 40 to about 94 percent, or of from about 50 to about 90 percent as compared to the amount of surfactants present in a toner particle prepared with the shell.

The choice of particular surfactants or combinations thereof, as well as the amounts of each to be used, are within the purview of those skilled in the art.

#### Initiators

In embodiments initiators may be added for formation of the latex polymer. Examples of suitable initiators include water soluble initiators, such as ammonium persulfate, sodium persulfate and potassium persulfate, and organic soluble initiators including organic peroxides and azo compounds including Vazo peroxides, such as VAZO 64™, 2-methyl 2-2'-azobis propanenitrile, VAZO 88™, 2-2'-azobis isobutyramid dehydrate, and combinations thereof. Other

water-soluble initiators which may be utilized include azoamidine compounds, for example 2,2'-azobis(2-methyl-N-phenylpropionamidine)dihydrochloride, 2,2'-azobis[N-(4-chlorophenyl)-2-methylpropionamidine]di-hydrochloride, 2,2'-azobis[N-(4-hydroxyphenyl)-2-methylpropionamidine]dihydrochloride, 2,2'-azobis[N-(4-amino-phenyl)-2-methylpropionamidine]tetrahydrochloride, 2,2'-azobis[2-methyl-N(phenylmethyl)propionamidine]dihydrochloride, 2,2'-azobis[2-methyl-N-2-propenylpropionamidine]dihydrochloride, 2,2'-azobis[N-(2-hydroxy-ethyl)-2-methylpropionamidine]dihydrochloride, 2,2'-azobis[2(5-methyl-2-imidazolin-2-yl)propane]dihydrochloride, 2,2'-azobis[2-(2-imidazolin-2-yl)propane]dihydrochloride, 2,2'-azobis[2-(4,5,6,7-tetrahydro-1H-1,3-diazepin-2-yl)propane]dihydrochloride, 2,2'-azobis[2-(3,4,5,6-tetrahydropyrimidin-2-yl)propane]dihydrochloride, 2,2'-azobis[2-(5-hydroxy-3,4,5,6-tetrahydropyrimidin-2-yl)propane]dihydrochloride, 2,2'-azobis{2-[1-(2-hydroxyethyl)-2-imidazolin-2-yl]propane}dihydrochloride, combinations thereof, and the like.

Initiators can be added in suitable amounts, such as from about 0.1 to about 8 weight percent of the monomers, in embodiments of from about 0.2 to about 5 weight percent of the monomers, in embodiments from about 0.5 to about 4 weight percent of the monomers.

## Chain Transfer Agents

In embodiments, chain transfer agents may also be utilized in forming the latex polymer. Suitable chain transfer agents include dodecanethiol, octanethiol, carbon tetrabromide, combinations thereof, and the like, in amounts from about 0.1 to about 10 percent of monomers, in embodiments from about 0.2 to about 5 percent by weight of monomers, and in embodiments from about 0.5 to about 3.5 percent by weight of monomers, to control the molecular weight properties of the latex polymer when emulsion polymerization is conducted in accordance with the present disclosure.

## Functional Monomers

In embodiments, it may be advantageous to include a functional monomer when forming the latex polymer and the particles making up the polymer. Suitable functional monomers include monomers having carboxylic acid functionality. Such monomers may be of the following formula (I):



(I)

where R1 is hydrogen or a methyl group; R2 and R3 are independently selected from alkyl groups containing from about 1 to about 12 carbon atoms or a phenyl group; n is from about 0 to about 20, in embodiments from about 1 to about 10. Examples of such functional monomers include beta carboxyethyl acrylate ( $\beta$ -CEA), poly(2-carboxyethyl) acrylate, 2-carboxyethyl methacrylate, combinations thereof, and the like. Other functional monomers which may be utilized include, for example, acrylic acid, methacrylic acid and its derivatives, and combinations of the foregoing.

In embodiments, the functional monomer having carboxylic acid functionality may also contain a small amount of metallic ions, such as sodium, potassium and/or calcium, to achieve better emulsion polymerization results. The metallic ions may be present in an amount from about 0.001 to about 10 percent by weight of the functional monomer having carboxylic acid functionality, in embodiments from about 0.5 to

about 5 percent by weight of the functional monomer having carboxylic acid functionality, in embodiments from about 0.75 to about 4 percent by weight of the functional monomer having carboxylic acid functionality.

5 Where present, the functional monomer may be added in amounts from about 0.01 to about 10 percent by weight of the total monomers, in embodiments from about 0.05 to about 5 percent by weight of the total monomers, and in embodiments from about 0.1 to about 3 percent by weight of total monomers.

Wax

Wax dispersions may also be added during formation of a latex polymer in an emulsion aggregation synthesis. Suitable waxes include, for example, submicron wax particles in the size range of from about 50 to about 1000 nanometers, in embodiments of from about 100 to about 500 nanometers in volume average diameter, suspended in an aqueous phase of water and an ionic surfactant, nonionic surfactant, or combinations thereof. Suitable surfactants include those described above. The ionic surfactant or nonionic surfactant may be present in an amount of from about 0.1 to about 20 percent by weight, and in embodiments of from about 0.5 to about 15 percent by weight of the wax.

The wax dispersion according to embodiments of the present disclosure may include, for example, a natural vegetable wax, natural animal wax, mineral wax, and/or synthetic wax. Examples of natural vegetable waxes include, for example, carnauba wax, candelilla wax, Japan wax, and bayberry wax. Examples of natural animal waxes include, for example, beeswax, punic wax, lanolin, lac wax, shellac wax, and spermaceti wax. Mineral waxes include, for example, paraffin wax, microcrystalline wax, montan wax, ozokerite wax, ceresin wax, petrolatum wax, and petroleum wax. Synthetic waxes of the present disclosure include, for example, Fischer-Tropsch wax, acrylate wax, fatty acid amide wax, silicone wax, polytetrafluoroethylene wax, polyethylene wax, polypropylene wax, and combinations thereof.

wax, polypropylene wax, and combinations thereof.

Examples of polypropylene and polyethylene waxes include those commercially available from Allied Chemical and Baker Petrolite, wax emulsions available from Michelman Inc. and the Daniels Products Company, EPOLENE N-15 commercially available from Eastman Chemical Products, Inc., VISCOL 550-P, a low weight average molecular weight polypropylene available from Sanyo Kasel K.K., and similar materials. In embodiments, commercially available polyethylene waxes possess a molecular weight (Mw) of from about 100 to about 5000, and in embodiments of from about 250 to about 2500, while the commercially available polypropylene waxes have a molecular weight of from about 200 to about 10,000, and in embodiments of from about 400 to about 5000.

In embodiments, the waxes may be functionalized. Examples of groups added to functionalize waxes include amines, amides, imides, esters, quaternary amines, and/or carboxylic acids. In embodiments, the functionalized waxes may be acrylic polymer emulsions, for example, JONCRYL 74, 89, 130, 537, and 538, all available from Johnson Diversey, Inc, or chlorinated polypropylenes and polyethylenes commercially available from Allied Chemical, Baker Petrolite Corporation and Johnson Diversey, Inc.

60 The wax may be present in an amount of from about 0.1 to about 30 percent by weight, and in embodiments from about 2 to about 20 percent by weight of the toner.

Colorants

65 The latex particles may be added to a colorant dispersion. The colorant dispersion may include, for example, submicron colorant particles having a size of, for example, from about 50

to about 500 nanometers in volume average diameter and, in embodiments, of from about 100 to about 400 nanometers in volume average diameter. The colorant particles may be suspended in an aqueous water phase containing an anionic surfactant, a nonionic surfactant, or combinations thereof. In embodiments, the surfactant may be ionic and may be from about 1 to about 25 percent by weight, and in embodiments from about 4 to about 15 percent by weight, of the colorant.

Colorants useful in forming toners in accordance with the present disclosure include pigments, dyes, mixtures of pigments and dyes, mixtures of pigments, mixtures of dyes, and the like. The colorant may be, for example, carbon black, cyan, yellow, magenta, red, orange, brown, green, blue, violet, or combinations thereof. In embodiments a pigment may be utilized. As used herein, a pigment includes a material that changes the color of light it reflects as the result of selective color absorption. In embodiments, in contrast with a dye which may be generally applied in an aqueous solution, a pigment generally is insoluble. For example, while a dye may be soluble in the carrying vehicle (the binder), a pigment may be insoluble in the carrying vehicle.

In embodiments wherein the colorant is a pigment, the pigment may be, for example, carbon black, phthalocyanines, quinacridones, red, green, orange, brown, violet, yellow, fluorescent colorants including RHODAMINE B™ type, and the like.

The colorant may be present in the toner of the disclosure in an amount of from about 1 to about 25 percent by weight of toner, in embodiments in an amount of from about 2 to about 15 percent by weight of the toner.

Exemplary colorants include carbon black like REGAL 330® magnetites; Mobay magnetites including MO8029™, MO8060™; Columbian magnetites; MAPICO BLACK™ and surface treated magnetites; Pfizer magnetites including CB4799™, CB5300™, CB5600™, MCX6369™; Bayer magnetites including, BAYFERROX 8600™, 8610™; Northern Pigments magnetites including, NP-604™, NP-608™; Magnox magnetites including TMB-100™, or TMB-104™, HELIOGEN BLUE L6900™, D6840™, D7080™, D7020™, PYLAM OIL BLUE™, PYLAM OIL YELLOW™, PIGMENT BLUE 1™ available from Paul Uhlrich and Company, Inc.; PIGMENT VIOLET 1™, PIGMENT RED 48™, LEMON CHROME YELLOW DCC 1026™, E.D. TOLUIDINE RED™ and BON RED C™ available from Dominion Color Corporation, Ltd., Toronto, Ontario; NOVAPERM YELLOW FGL™, HOSTAPERM PINK E™ from Hoechst; and CINQUASIA MAGENTA™ available from E.I. DuPont de Nemours and Company. Other colorants include 2,9-dimethyl-substituted quinacridone and anthraquinone dye identified in the Color Index as Cl 60710, Cl Dispersed Red 15, diazo dye identified in the Color Index as Cl 26050, Cl Solvent Red 19, copper tetra(octadecyl sulfonamido) phthalocyanine, x-copper phthalocyanine pigment listed in the Color Index as Cl 74160, Cl Pigment Blue, Anthrathrene Blue identified in the Color Index as Cl 69810, Special Blue X-2137, diarylide yellow 3,3-dichlorobenzidine acetoacetanilides, a monoazo pigment identified in the Color Index as Cl 12700, Cl Solvent Yellow 16, a nitrophenyl amine sulfonamide identified in the Color Index as Foron Yellow SE/GLN, Cl Dispersed Yellow 33, 2,5-dimethoxy-4-sulfonanilide phenylazo-4'-chloro-2,5-dimethoxy acetoacetanilide, Yellow 180 and Permanent Yellow FGL. Organic soluble dyes having a high purity for the purpose of color gamut which may be utilized include Neopen Yellow 075, Neopen Yellow 159, Neopen Orange 252, Neopen Red 336, Neopen Red 335, Neopen Red 366, Neopen Blue 808, Neopen Black X53, Neopen Black X55, wherein the dyes are

selected in various suitable amounts, for example from about 0.5 to about 20 percent by weight, in embodiments, from about 5 to about 18 weight percent of the toner.

In embodiments, colorant examples include Pigment Blue 15:3 having a Color Index Constitution Number of 74160, Magenta Pigment Red 81:3 having a Color Index Constitution Number of 45160:3, Yellow 17 having a Color Index Constitution Number of 21105, and known dyes such as food dyes, yellow, blue, green, red, magenta dyes, and the like.

In other embodiments, a magenta pigment, Pigment Red 122 (2,9-dimethylquinacridone), Pigment Red 185, Pigment Red 192, Pigment Red 202, Pigment Red 206, Pigment Red 235, Pigment Red 269, combinations thereof, and the like, may be utilized as the colorant. Pigment Red 122 (sometimes referred to herein as PR-122) has been widely used in the pigmentation of toners, plastics, ink, and coatings, due to its unique magenta shade.

#### pH Adjustment Agent

In some embodiments a pH adjustment agent may be added to control the rate of the emulsion aggregation process. The pH adjustment agent utilized in the processes of the present disclosure can be any acid or base that does not adversely affect the products being produced. Suitable bases can include metal hydroxides, such as sodium hydroxide, potassium hydroxide, ammonium hydroxide, and optionally combinations thereof. Suitable acids include nitric acid, sulfuric acid, hydrochloric acid, citric acid, acetic acid, and optionally combinations thereof. The amount of the base addition may thus be of from about 0.1% wt/wt to about 20% wt/wt, in other embodiments from about 0.2% wt/wt to about 10% wt/wt, in further embodiments from about 0.5% wt/wt to about 5% wt/wt.

#### Coagulants

In embodiments, a coagulant may be added during or prior to aggregating the latex and the aqueous colorant dispersion. The coagulant may be added over a period of time from about 1 minute to about 60 minutes, in embodiments from about 1.25 minutes to about 20 minutes, in embodiments from about 2 minutes to about 15 minutes, depending on the processing conditions.

Examples of suitable coagulants include polyaluminum halides such as polyaluminum chloride (PAC), or the corresponding bromide, fluoride, or iodide, polyaluminum silicates such as polyaluminum sulfo silicate (PASS), and water soluble metal salts including aluminum chloride, aluminum nitrite, aluminum sulfate, potassium aluminum sulfate, calcium acetate, calcium chloride, calcium nitrite, calcium oxydate, calcium sulfate, magnesium acetate, magnesium nitrate, magnesium sulfate, zinc acetate, zinc nitrate, zinc sulfate, combinations thereof, and the like. One suitable coagulant is PAC, which is commercially available and can be prepared by the controlled hydrolysis of aluminum chloride with sodium hydroxide. Generally, PAC can be prepared by the addition of two moles of a base to one mole of aluminum chloride. The species is soluble and stable when dissolved and stored under acidic conditions if the pH is less than about 5. The species in solution is believed to contain the formula  $Al_{13}O_4(OH)_{24}(H_2O)_{12}$  with about 7 positive electrical charges per unit.

In embodiments, suitable coagulants include a polymetal salt such as, for example, polyaluminum chloride (PAC), polyaluminum bromide, or polyaluminum sulfosilicate. The polymetal salt can be in a solution of nitric acid, or other diluted acid solutions such as sulfuric acid, hydrochloric acid, citric acid or acetic acid. The coagulant may be added in amounts from about 0.01 to about 5 percent by weight of the toner, in embodiments from about 0.1 to about 3 percent by

## 11

weight of the toner, and in embodiments from about 0.5 to about 2 percent by weight of the toner.

## Aggregating Agents

Any aggregating agent capable of causing complexation might be used in forming toner of the present disclosure. Both alkali earth metal or transition metal salts can be utilized as aggregating agents. In embodiments, alkali (II) salts can be selected to aggregate sodium sulfonated polyester colloids with a colorant to enable the formation of a toner composite. Such salts include, for example, beryllium chloride, beryllium bromide, beryllium iodide, beryllium acetate, beryllium sulfate, magnesium chloride, magnesium bromide, magnesium iodide, magnesium acetate, magnesium sulfate, calcium chloride, calcium bromide, calcium iodide, calcium acetate, calcium sulfate, strontium chloride, strontium bromide, strontium iodide, strontium acetate, strontium sulfate, barium chloride, barium bromide, barium iodide, and optionally combinations thereof. Examples of transition metal salts or anions which may be utilized as aggregating agent include acetates of vanadium, niobium, tantalum, chromium, molybdenum, tungsten, manganese, iron, ruthenium, cobalt, nickel, copper, zinc, cadmium or silver; acetoacetates of vanadium, niobium, tantalum, chromium, molybdenum, tungsten, manganese, iron, ruthenium, cobalt, nickel, copper, zinc, cadmium or silver; sulfates of vanadium, niobium, tantalum, chromium, molybdenum, tungsten, manganese, iron, ruthenium, cobalt, nickel, copper, zinc, cadmium or silver; and aluminum salts such as aluminum acetate, aluminum halides such as polyaluminum chloride, combinations thereof, and the like. The amount of the aggregating agent addition may thus be of from about 0.01% wt/wt to about 1% wt/wt, in other embodiments from about 0.1% wt/wt to about 0.5% wt/wt, in further embodiments from about 0.15% wt/wt to about 0.3% wt/wt.

## Reaction Conditions

In the emulsion aggregation process, the reactants may be added to a suitable reactor, such as a mixing vessel. The resulting blend of latex, optionally in a dispersion, CCA, optionally in dispersion, optional colorant dispersion, optional wax, optional coagulant, and optional aggregating agent, may then be stirred and heated to a temperature at or above the glass transition temperature (T<sub>g</sub>) of the latex, in embodiments from about 30° C. to about 70° C., in embodiments of from about 40° C. to about 65° C., in embodiments from about 45° C. to about 60° C., for a period of time from about 0.2 hours to about 6 hours, in embodiments from about 0.3 hours to about 5 hours, in embodiments from about 0.5 hours to about 3 hours, resulting in toner aggregates of from about 3 microns to about 15 microns in volume average diameter, in embodiments of from about 4 microns to about 8 microns in volume average diameter, in embodiments from about 5 microns to about 7 microns in volume average diameter.

Once the desired final size of the toner particles is achieved, the pH of the mixture may be adjusted with a base, to freeze the growth process of the particle, to a value of no higher than 7 or no higher than 4.5. In specific embodiments, the pH is adjusted to from about 3.5 to about 7, or from about 4 to about 6.5. The base may include any suitable base such as, for example, alkali metal hydroxides such as, for example, sodium hydroxide, potassium hydroxide, and ammonium hydroxide. The alkali metal hydroxide may be added in amounts from about 0.1 to about 30 percent by weight of the mixture, in embodiments from about 0.5 to about 15 percent by weight of the mixture.

The toner particles may be subsequently coalesced. Coalescing may include stirring and heating at a temperature of

## 12

from about 80° C. to about 100° C., in embodiments from about 90° C. to about 99° C., for a period of from about 0.5 hours to about 12 hours, and in embodiments from about 1 hour to about 6 hours. Coalescing may be accelerated by 5 additional stirring. The particles are coalesced until the desired circularity or roundness of the particles are reached, for example, from about 0.960 to about 0.990, or from about 0.965 to about 0.975.

The pH of the mixture may then be lowered to from about 10 3.5 to about 6, in embodiments from about 3.7 to about 5.5, with, for example, an acid to coalesce the toner aggregates. Suitable acids include, for example, nitric acid, sulfuric acid, hydrochloric acid, citric acid or acetic acid. The amount of acid added may be from about 0.1 to about 30 percent by 15 weight of the mixture, and in embodiments from about 1 to about 20 percent by weight of the mixture.

The mixture is cooled in a cooling or freezing step. Cooling may be at a temperature of from about 20° C. to about 40° C., in embodiments from about 22° C. to about 30° C. over a 20 period time from about 1 hour to about 8 hours, and in embodiments from about 1.5 hours to about 5 hours.

In embodiments, cooling a coalesced toner slurry includes 25 quenching by adding a cooling medium such as, for example, ice, dry ice and the like, to effect rapid cooling to a temperature of from about 20° C. to about 40° C., and in embodiments of from about 22° C. to about 30° C. Quenching may be feasible for small quantities of toner, such as, for example, less than about 2 liters, in embodiments from about 0.1 liters to about 1.5 liters. For larger scale processes, such as for 30 example greater than about 10 liters in size, rapid cooling of the toner mixture may not be feasible or practical, neither by the introduction of a cooling medium into the toner mixture, nor by the use of jacketed reactor cooling.

## Washing

The toner slurry may then be washed. Washing may be 35 carried out at a pH of from about 7 to about 12, and in embodiments at a pH of from about 9 to about 11. The washing may be at a temperature of from about 30° C. to about 70° C., in embodiments from about 40° C. to about 67° 40 C. The washing may include filtering and re-slurrying a filter cake including toner particles in deionized water. The filter cake may be washed one or more times by deionized water, or washed by a single deionized water wash at a pH of about 4 45 wherein the pH of the slurry is adjusted with an acid, and followed optionally by one or more deionized water washes. In embodiments, the particles may be washed about three times with water.

For example, in embodiments, toner particles may be 50 washed in 40° C. deionized water, filtered, re-slurried with HCl acid addition, filtered, and re-slurried in fresh deionized water. The washes may continue until the solution conductivity of the filtrate is measured to be low (less than 10 microsiemens per centimeter), which indicates that the ion content is significantly reduced and will not interfere with the metal, 55 in embodiments zinc, treatment.

The washing of the toner particles with the metal ion solution may take place at a temperature of from about 30° C. to about 50° C. The metal ion solution, in embodiments including zinc, is added dropwise to the slurry in an amount of from 60 about 1 to about 120 drops. The metal ion solution is added dropwise to the slurry at a rate of from about 1 drops/min to about 120 drops/min, in embodiments from about 5 drops/min to about 100 drops/min, in embodiments from about 10 drops/min to about 60 drops/min, and mixed for a period of 65 from about 0.5 hours to about 1.5 hours, in embodiments from about 0.75 hours to about 1.25 hours, in embodiments about 1 hour. During this time of mixing, the slurry is slightly heated

## 13

from about 20° C. to about 60° C., in other embodiments from about 30° C. to about 55° C., in further embodiments from about 35° C. to about 45° C. The zinc attaches to the toner surface in a controlled manner without aggregating the particles together.

In embodiments, the particles may then be subjected to an additional washing step including a metal in solution to enhance their charging characteristics. An increase in the amount of certain metal based charging agents, in embodiments zinc salicylate or other similar agent, on the surface of a toner particle may increase the charging of the toner particles. Thus, in accordance with the present disclosure, a washing step including such a metal may increase the charging of the toner particles.

## Treatment of Coalesced Particles

After coalescing, the process of the present embodiments subject the toner particles one or more additional treatment steps to improve the charging properties of the toner particles. In embodiments, the toner particles are given a final wash, as described above, and re-slurried in water. In embodiments, a toner wet cake may be re-dispersed in water, in embodiments deionized water, and heated to a temperature of from about from about 20° C. to about 50° C., in embodiments from about 35° C. to about 45° C., in other embodiments about 40° C. A charge control agent dispersion is then added to the slurry.

The dispersion may comprise a metal-based charging agent, such as for example, zinc salicylate, chromium salicylate, aluminum salicylate or other metal based charge control agents. The dispersion is added thereto and mixed so that the metal salicylate attaches to the surface of the toner particles. Suitable sources of metal charging agents in this step may include zinc acetate, zinc butyrate, zinc chlorate, zinc chloride, zinc bromide, zinc citrate, zinc fluoride, zinc salicylate, aluminum salicylate, zinc fluoride tetrahydrate, zinc 3,5-di-tertiarybutylsalicylic acid, aluminum 3,5-di-tertiarybutylsalicylic acid combinations thereof, and the like. In accordance with the present disclosure, the dispersion may incorporate any suitable CCA as disclosed herein. In specific embodiments, a CCA such as 3,5-di-tert-butylsalicylic acid or a mixture of hydroxyaluminum-bis[2-hydroxy-3,5-di-tert-butylbenzoate] and 3,5-di-tert-butylsalicylic acid may be added to improve charging in all zones and the life of the toner. In embodiments, the charge control total solids in dispersion is added in an amount of from about 0.1 to about 10 percent, or from about 0.5 to about 8 percent, or from about 1 to about 6 percent by weight of CCA, the total weight of the particle batch, including all components that are being mixed together in the reactor. In embodiments, the slurry is solids in the batch comprising from about 10 to about 20% of solids total. Thus, in embodiments, the charge control solids in the dispersion is added in an amount of from about 0.05 to about 10 percent, or from about 2.0 to about 5.0 percent by weight of the total solids weight in the slurry.

The slurry comprising the charge control agent dispersion is next heated to above the Tg of the latex, for example, from about 40 to about 65° C., or from about 45 to about 55° C., and mixed with constant high shearing for up to one hour, for example, from about 2 to about 120 minutes, or from about 20 to about 60 minutes. The slurry is mixed at a speed of from about 1,000 to about 10,000 RPM, or from about 4,000 to about 7,000 RPM.

The treated toner may then be filtered and redispersed in deionized water, then freeze dried for about 48 hours. The drying may be continued until the moisture level of the particles is of from about 0% to about 1% by weight, in embodiments from about 0.1% to about 0.7% by weight. The toner

## 14

particles produced possess a triboelectric charge of from about -2 µC/g to about -60 µC/g, or from about -10 µC/g to about -45 µC/g, or from about -20 µC/g to about -35 µC/g. Additives

5 Further optional additives which may be combined with a toner include any additive to enhance the properties of toner compositions. Included are surface additives, color enhancers, etc. Surface additives that can be added to the toner compositions after washing or drying include, for example, 10 metal salts, metal salts of fatty acids, colloidal silicas, metal oxides, strontium titanates, combinations thereof, and the like, which additives are each usually present in an amount of from about 0.1 to about 10 weight percent of the toner, in embodiments from about 0.5 to about 7 weight percent of the toner. Examples of such additives include, for example, those 15 disclosed in U.S. Pat. Nos. 3,590,000, 3,720,617, 3,655,374 and 3,983,045, the disclosures of each of which are hereby incorporated by reference in their entirety. Other additives include zinc stearate and AEROSIL R972™ available from 20 Degussa. The coated silicas of U.S. Pat. No. 6,190,815 and U.S. Pat. No. 6,004,714, the disclosures of each of which are hereby incorporated by reference in their entirety, can also be selected in amounts, for example, of from about 0.05 to about 5 percent by weight of the toner, in embodiments from about 25 0.1 to about 2 percent by weight of the toner. These additives can be added during the aggregation or blended into the formed toner product.

Toner particles produced utilizing a latex of the present disclosure may have a size of about 1 micron to about 20 30 microns, in embodiments about 2 microns to about 15 microns, in embodiments about 3 microns to about 7 microns. Toner particles of the present disclosure may have a circularity of from about 0.9 to about 0.99, in embodiments from about 0.92 to about 0.98.

35 Following the methods of the present disclosure, toner particles may be obtained having several advantages compared with conventional toners: (1) increase in the robustness of the particles' triboelectric charging, which reduces toner defects and improves machine performance; (2) easy to 40 implement, no major changes to existing aggregation/coalescence processes; and (3) increase in productivity and reduction in unit manufacturing cost (UMC) by reducing the production time and the need for rework (quality yield improvement).

## 45 Uses

Toner in accordance with the present disclosure can be used in a variety of imaging devices including printers, copy machines, and the like. The toners generated in accordance with the present disclosure are excellent for imaging processes, especially xerographic processes and are capable of providing high quality colored images with excellent image resolution, acceptable signal-to-noise ratio, and image uniformity. Further, toners of the present disclosure can be selected for electrophotographic imaging and printing processes such as digital imaging systems and processes.

Developer compositions can be prepared by mixing the toners obtained with the processes disclosed herein with known carrier particles, including coated carriers, such as steel, ferrites, and the like. Such carriers include those disclosed in U.S. Pat. Nos. 4,937,166 and 4,935,326, the entire disclosures of each of which are incorporated herein by reference. The carriers may be present from about 2 percent by weight of the toner to about 8 percent by weight of the toner, in embodiments from about 4 percent by weight to about 6 55 percent by weight of the toner. The carrier particles can also include a core with a polymer coating thereover, such as polymethylmethacrylate (PMMA), having dispersed therein

## 15

a conductive component like conductive carbon black. Carrier coatings include silicone resins such as methyl silsesquioxanes, fluoropolymers such as polyvinylidene fluoride, mixtures of resins not in close proximity in the triboelectric series such as polyvinylidene fluoride and acrylics, thermosetting resins such as acrylics, combinations thereof and other known components.

Development may occur via discharge area development. In discharge area development, the photoreceptor is charged and then the areas to be developed are discharged. The development fields and toner charges are such that toner is repelled by the charged areas on the photoreceptor and attracted to the discharged areas. This development process is used in laser scanners.

Development may be accomplished by the magnetic brush development process disclosed in U.S. Pat. No. 2,874,063, the disclosure of which is hereby incorporated by reference in its entirety. This method entails the carrying of a developer material containing toner of the present disclosure and magnetic carrier particles by a magnet. The magnetic field of the magnet causes alignment of the magnetic carriers in a brush like configuration, and this "magnetic brush" is brought into contact with the electrostatic image bearing surface of the photoreceptor. The toner particles are drawn from the brush to the electrostatic image by electrostatic attraction to the discharged areas of the photoreceptor, and development of the image results. In embodiments, the conductive magnetic brush process is used wherein the developer includes conductive carrier particles and is capable of conducting an electric current between the biased magnet through the carrier particles to the photoreceptor.

## Imaging

Imaging methods are also envisioned with the toners disclosed herein. Such methods include, for example, some of the above patents mentioned above and U.S. Pat. Nos. 4,265,990, 4,584,253 and 4,563,408, the entire disclosures of each of which are incorporated herein by reference. The imaging process includes the generation of an image in an electronic printing magnetic image character recognition apparatus and thereafter developing the image with a toner composition of the present disclosure. The formation and development of images on the surface of photoconductive materials by electrostatic means is well known. The basic xerographic process involves placing a uniform electrostatic charge on a photoconductive insulating layer, exposing the layer to a light and shadow image to dissipate the charge on the areas of the layer exposed to the light, and developing the resulting latent electrostatic image by depositing on the image a finely-divided electroscopic material, for example, toner. The toner will normally be attracted to those areas of the layer, which retain a charge, thereby forming a toner image corresponding to the latent electrostatic image. This powder image may then be transferred to a support surface such as paper. The transferred image may subsequently be permanently affixed to the support surface by heat. Instead of latent image formation by uniformly charging the photoconductive layer and then exposing the layer to a light and shadow image, one may form the latent image by directly charging the layer in image configuration. Thereafter, the powder image may be fixed to the

## 16

photoconductive layer, eliminating the powder image transfer. Other suitable fixing means such as solvent or overcoating treatment may be substituted for the foregoing heat fixing step.

Various exemplary embodiments encompassed herein include a method of imaging which includes generating an electrostatic latent image on an imaging member, developing a latent image, and transferring the developed electrostatic image to a suitable substrate.

While the description above refers to particular embodiments, it will be understood that many modifications may be made without departing from the spirit thereof. The accompanying claims are intended to cover such modifications as would fall within the true scope and spirit of embodiments herein.

The presently disclosed embodiments are, therefore, to be considered in all respects as illustrative and not restrictive, the scope of embodiments being indicated by the appended claims rather than the foregoing description. All changes that come within the meaning of and range of equivalency of the claims are intended to be embraced therein.

## EXAMPLES

The example set forth herein below and is illustrative of different compositions and conditions that can be used in practicing the present embodiments. All proportions are by weight unless otherwise indicated. It will be apparent, however, that the embodiments can be practiced with many types of compositions and can have many different uses in accordance with the disclosure above and as pointed out hereinabove.

## Example 1

## Formation of Toner Particles

Styrene/Butylacrylate latex polymer was mixed with low melt paraffin wax and carbon black and cyan pigment in the appropriate ratios. Polyaluminum chloride was then added to the system and the mix homogenized for a period of time. Once homogenized, the reactor contents were heated to near the glass transition temperature of the polymer for a period of time until the particle reached desired size. Once the aggregate was at the appropriate size (6.2  $\mu\text{m}$ ), the reactor was held at temperature for a period of time and then a base was added to further freeze the particle size and adjust the pH higher in alkalinity. Once frozen, the particle batch temperature was raised to no less than 90° C. and the pH was adjusted to no higher than 5.0. The batch then coalesced for a period of time until a circularity (roundness) of the particle was 0.970 or greater. The batch was then cooled, pH adjusted up, washed and then dried. Dried particle was then taken and blended with the optimized additive formulation to produce a toner. This resulted in a homogeneous dispersion of CCA polymer in the particle.

Table 1 provides the experimental results of the toner particles prepared with and without shell to improve the incorporate of zinc charge control agent and reduce levels of surfactant.

TABLE 1

| Run | Description           | Bontron<br>E-84 (LC) | Particle<br>(ICP)         |                           | Surfactant Amount<br>(LC/MS)     |                              | Toner Parent<br>(XPS) |
|-----|-----------------------|----------------------|---------------------------|---------------------------|----------------------------------|------------------------------|-----------------------|
|     |                       | Bontron<br>E-84 (%)  | Al<br>( $\mu\text{g/g}$ ) | Zn<br>( $\mu\text{g/g}$ ) | Dowfax 2A<br>( $\mu\text{g/g}$ ) | Tayca<br>( $\mu\text{g/g}$ ) | Zn<br>(attachment %)  |
| 1   | 0% CCA-latex in shell | 0                    | 791                       | 1.2                       | 107                              | 1409                         | 0                     |

TABLE 1-continued

| Run | Description                        | Bontron   | Particle            | Surfactant Amount   | Toner Parent        |                     |                |
|-----|------------------------------------|-----------|---------------------|---------------------|---------------------|---------------------|----------------|
|     |                                    | E-84 (LC) | (ICP)               | (LC/MS)             | (XPS)               |                     |                |
|     |                                    | Bontron   | Al                  | Zn                  | Dowfax 2A           | Tayca               | Zn             |
|     |                                    | E-84 (%)  | ( $\mu\text{g/g}$ ) | ( $\mu\text{g/g}$ ) | ( $\mu\text{g/g}$ ) | ( $\mu\text{g/g}$ ) | (attachment %) |
| 2   | 0% CCA-latex in core, no shell     | 0         | 931                 | ND                  | 26                  | 510                 | 0              |
| 3   | 20% Zn CCA-latex in shell          | 0.15      | 843                 | 113                 | 201                 | 1761                | 0.11           |
| 4   | 20% Zn CCA-latex in core, no shell | 0.39      | 872                 | 290                 | 126                 | 1395                | 0.28           |

From Table 1, reduction in surfactant in the particle without shell is observed as well as an increase in total zinc charge control agent in the particle without shell as compared to the particle with shell. Moreover, the particle with 20% zinc charge control with shell showed a reduced total amount of retained zinc charge control agent while the shell-less toner particle showed higher bulk zinc charge control agent and XPS (surface) zinc levels.

It will be appreciated that various of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

What is claimed is:

1. A toner comprising

shell-less toner particles comprising

a core portion comprising a resin, wax and colorant, and a charge control agent distributed homogeneously throughout the core portion, wherein a bulk level of the charge control agent in the core portion is from about 0.1 to about 50 percent by weight of the total weight of the toner particle and a surface level of the charge control agent on the core portion is from about 0.01 to about 10 percent by weight of the total weight of the toner particle.

2. The toner of claim 1, wherein toner is an emulsion aggregation toner.

3. The toner of claim 1, wherein the charge control agent is selected from the group consisting of metal complexes of alkyl derivatives of acids such as salicylic acid, dicarboxylic acid derivatives, benzoic acid, oxynaphthoic acid, and sulfonic acids, or other complexes such as polyhydroxyalcanoate quaternary phosphonium trihalozincate, and metal complexes of dimethyl sulfoxide, and mixtures thereof.

4. The toner of claim 1, wherein the charge control agent is present in an amount of from about 0.01 to about 15 percent by weight of the total weight of the toner particle.

5. The toner of claim 1 having a triboelectric charge of from about -5 to about -60 uC/gm in A zone.

6. The toner of claim 1, wherein the bulk level of the charge control agent is increased from about 5 to about 30 percent as compared to a bulk level of a toner particle prepared with the shell.

7. The toner of claim 1, wherein the surface level of the charge control agent is increased from about 0.1 to about 15 percent as compared to a surface level of a toner particle prepared with the shell.

8. The toner of claim 1, wherein the toner particles further comprise one or more surface additives.

9. The toner of claim 1, wherein the toner particles have an average particle size of from about 4.5 to about 7.5 um.

10. A toner comprising  
shell-less toner particles comprising  
a core portion comprising a resin, wax and colorant,  
a charge control agent distributed homogeneously  
throughout the core portion, and  
a residual surfactant on a surface of the core portion,  
wherein an amount of surfactant present in the toner  
particle is from about 20 to about 2500 ppm of the  
toner particle.

11. The toner of claim 10, wherein the amount of surfactant present in the toner particle is reduced as compared to an amount of surfactant present in a toner particle prepared with the shell.

12. The toner of claim 10, wherein amount of surfactant present in the toner particle is decreased from about 80 percent to about 30 percent as compared to an amount of surfactant present in a toner particle prepared with the shell.

13. A process for producing toner comprising:  
adding and mixing a colorant, a wax, and a charge control  
agent to an emulsion comprising at least one resin to  
form toner particles;  
aggregating the particles to form aggregated particles; and  
coalescing the aggregated particles to form shell-less toner  
particles comprising

a core portion comprising a resin, wax and colorant, and  
a charge control agent distributed homogeneously  
throughout the core portion, wherein a bulk level of  
the charge control agent in the core portion is from  
about 0.1 to about 50 percent by weight of the total  
weight of the toner particle and a surface level of the  
charge control agent on the core portion is from about  
0.01 to about 10 percent by weight of the total weight  
of the toner particle.

14. The process of claim 13 further comprising washing the  
shell-less toner particles.

15. The process of claim 13, wherein toner is an emulsion aggregation toner.

16. The process of claim 13, wherein the charge control agent is selected from the group consisting of a zinc complex of 3,5-di-tert-butylsalicylic acid in powder form, a mixture of hydroxyaluminium-bis[2-hydroxy-3,5-di-tert-butylbenzoate] and 3,5-di-tert-butylsalicylic acid, a calcium complex

**19**

of 3,5-di-tert-butylsalicylic acid, a zirconium complex of 3,5-di-tert-butylsalicylic acid, an aluminum complex of 3,5-di-tert-butylsalicylic acid, mixtures thereof.

**17.** The process of claim **13**, wherein the toner has a triboelectric charge of from about -5 to about -60 uC/gm. 5

**20**

\* \* \* \*